

March 6, 1973

D. J. FORST

3,719,493

RAPID COLOR PROCESSING

Filed March 24, 1971

3 Sheets-Sheet 1



FIG. 1



FIG. 3



FIG. 2

DONALD J. FORST  
INVENTOR.

BY *David E. Brook*

ATTORNEY.

March 6, 1973

D. J. FORST

3,719,493

RAPID COLOR PROCESSING

Filed March 24, 1971

3 Sheets-Sheet 2



FIG. 4

DONALD J. FORST  
INVENTOR

BY *David E. Brook*  
ATTORNEY

March 6, 1973

D. J. FORST

3,719,493

RAPID COLOR PROCESSING

Filed March 24, 1971

3 Sheets-Sheet 3



FIG. 5



FIG. 6

DONALD J. FORST  
INVENTOR

BY *David E. Brook*

ATTORNEY.

**1**

3,719,493

**RAPID COLOR PROCESSING**Donald J. Forst, Webster, N.H., assignor to Itek  
Corporation, Lexington, Mass.Continuation-in-part of applications Ser. No. 699,576, Jan.  
22, 1968, and Ser. No. 831,226, June 6, 1969, both now  
abandoned. This application Mar. 24, 1971, Ser. No.  
127,689

Int. Cl. G03c 7/00

U.S. Cl. 96—55

41 Claims

**ABSTRACT OF THE DISCLOSURE**

This disclosure relates to improved reversal color processing which includes hardening the color film emulsion subsequent to developing the negative image of the film. The improved process permits the use of relatively high temperatures in the steps subsequent to the hardening step thus permitting more rapid film processing while maintaining good color properties. The process steps include first developing the negative image, subsequently hardening the emulsion to be stable to water at 140° F. or above, and then completing processing with steps such as color developing, fixing and stabilizing at elevated temperatures.

Also described are improved processing steps for negative color processing and compositions useful therefor.

Improved silver negative development is realized by use of methylhydroquinone. Acidification of the film emulsion subsequent to negative development is enhanced by swell-suppressing agents. The use of chelating agents in the stabilizing step substantially eliminates sludge formation. A fixing solution containing soluble thiocyanates and soluble thiosulfates gives improved results. The use of one or more viscous solutions to improve processing is described.

Apparatus for accomplishing the improved color processing is also described.

The invention herein described was made in the course of or under a contract or subcontract thereunder with the United States Government, Department of Defense.

**CROSS REFERENCE TO RELATED APPLICATIONS**

This application is a continuation-in-part of Forst, Ser. No. 699,576, filed Jan. 22, 1968 and Forst, Ser. No. 831,226, filed June 6, 1969, both abandoned.

**BACKGROUND OF THE INVENTION****(1) Field of the invention**

This invention relates to rapid, reversal and negative color processing.

**(2) Description of the prior art**

Many attempts have been made to reduce the time required for processing of multilayer, multicolor photographic elements to positive color images, i.e. reversal color processing, or to negative color images, i.e. negative color processing. In reversal color processing, the processing steps include first developing to form a negative black and white image; the photographic element is then fogged or re-exposed and color-developed with a color-forming coupler which reacts with the oxidized developer to form an appropriate dye image corresponding to the positive silver image formed. Finally the silver images and remaining silver halide are removed by bleaching and fixing to leave the color image. In negative color processing, the processing steps involve color developing the exposed film, followed by bleaching out of the silver image, and fixing of the silver halide to leave the color image.

Typical prior art color processes wherein first development is carried out prior to a hardening step are known as

**2**

the Kodak Color Process C-22 (negative) and the Kodak Ektachrome Process E-1 (reversal). These processes are well known and have been described in numerous Kodak technical publications as well as in Eaton, *Photographic Chemistry*, 2nd ed., 1965 at page 92 et seq. The steps subsequent to hardening in these processes are carried out at temperatures of about 75° F., and these processes take around 60 minutes to complete.

A newer reversal process, the Kodak ME-4 process, uses higher temperatures to reduce total processing time. In this process, however, there is no hardening step after first development. Also, this process uses processing temperatures of about 100° F. so that the color properties of the processed image will not be harmed by higher temperatures. Total processing time is approximately 27 minutes.

The attempts to reduce the overall processing time required have resulted in rapid processing methods which, however, sacrifice color balance and soften film emulsion, i.e. lower film abrasion resistance, in particular. A solution to the problem of film abrasion resistance has been suggested by the use of hardening agents for the film emulsions, for example as described in U.S. Pat. 3,168,400 to Blackmer et al. In the said patent, the film emulsion is subjected to treatment with an aqueous solution of an aldehyde prior to photographic development but subsequent to photoexposure. However, the prehardening leads to considerable difficulty in maintenance of color balance. A major difficulty in processing color emulsions is the problem of maintaining the sensitometric characteristics during the first stage of development. Major gamma and speed shifts in one or more of the emulsion layers can alter the color balance. Such alterations are related to the chemical and diffusion rates of development within each layer. Another effect of accelerated development is the softening of the emulsions as a result of the use of elevated temperatures and high pH often associated with high energy developers. The hardeners are used to reduce these effects. However, the hardeners normally harden the top layer (the yellow dye forming layer in Ektachrome film) to a greater degree than the second and subsequent layers (the magenta and cyan layers). Thus, when the film is immersed in the first developer, reaction on the first layer is not as fast as that on the subsequent layers. This generally causes severe shifts in gamma and speed, and tends to alter the color balance. Such alteration cannot be wholly compensated for in the remaining stages of the process since the original sensitometric characteristics have been altered.

Generally, the maximum temperatures heretofore utilized in the various processing steps do not substantially exceed 100° F. and usually are somewhat lower than 100° F. since the use of high temperatures, particularly with significant changes of pH in the various steps, leads to rapid change in the swell of the film emulsion, particularly gelatin which is most common in film. As is commonly known, gelatin swell leads to image distortion.

A further difficulty encountered in reversal color processing is the need for numerous water washing steps because of water volume requirements which, in automated processing apparatus, creates the need for additional baths in the processing sequence, and results in more complex and larger apparatus. Most attempts to reduce the processing time have been directed to elimination of large volumes of wash water which have been only partially, if at all, successful.

**SUMMARY OF THE INVENTION**

It has now been unexpectedly found that rapid color processing can be accomplished by first developing the negative image in a multilayer film and subsequently rendering the film stable to water at a temperature of at

least about 140° F., followed by the usual processing. This sequence of steps avoids the difficulties inherent in first hardening the film emulsion prior to negative development. Specifically, better color balance is obtained since the sensitometric characteristics of the various emulsion layers of the film are more easily controlled than is possible with emulsions which are prehardened. However, one skilled in the art will recognize that a limited amount of hardening prior to first development is permissible, either in the processing or in the manufacture of the film, so long as this prehardening does not substantially interfere with the color balance and create other above mentioned problems in the color processing.

After the development of the negative image, the film emulsion is rendered stable to water at a temperature of at least about 140° F., and preferably at least about 180° F., when rapid, high temperature color processing is desired. The upper limit of temperature to which the hardened film is stable is limited only by the boiling temperature of the treating solution, i.e. for practical considerations, about 212° F.

For the purpose of this disclosure, the word "stable" means that the film emulsion undergoes no change adverse to photographic processing. Such changes primarily include softening of the film emulsion, which leads to distortion of the color image, and film reticulation, the most pronounced effect of which is separation of the film emulsion from the support material.

In its preferred form, the invention contemplates the use of aldehyde hardeners, especially dialdehyde hardeners.

Although it is preferred to stabilize the film subsequent to first development, it will be understood that the stabilizing step may be used at any point in the subsequent processing of the film, e.g., subsequent to the color developing step in reversal color processing. The stabilization subsequent to the first development is preferred since it permits shorter processing time in each of the subsequent steps by allowing the use of higher temperatures than are normally employed.

For the purpose of this disclosure, the term "rapid processing" or "high-speed processing" refers to processing wherein at least one, and preferably several or all, of the steps subsequent to hardening are carried out at a temperature in excess of 100° F., usually above 110° F., and wherein total processing time is not more than about 30 minutes.

#### BRIEF DESCRIPTION OF THE DRAWINGS

FIG. 1 illustrates a deep tank continuous processor for rapidly processing color-reversal film.

FIG. 2 illustrates a deep tank continuous processor for rapidly processing negative color film.

FIG. 3 illustrates a modified deep tank continuous processor for rapidly processing color-reversal film using a viscous color developer.

FIG. 4 illustrates sensitometric curves for a reversal color film processed according to this invention.

FIG. 5 illustrates sensitometric curves for a negative color film processed according to this invention.

FIG. 6 illustrates sensitometric curves for a negative color film processed according to a prior art method.

#### REVERSAL COLOR PROCESSING

In reversal color processing, the film emulsion subsequent to the first development step is alkaline and therefore must be acidified prior to aldehyde hardening to prevent reaction of the dye coupler in the film emulsion with the aldehyde. The efficiency of the acidification step is particularly enhanced by the presence of swell-suppressing agents in the acid bath. During the acidification process, the excess developer and oxidized developer are removed from the film emulsion, which removal is also enhanced by the swell-suppressing agents.

After the developed film is acidified, it is then hardened

with the aldehyde hardener, after which the excess aldehyde must be removed prior to the color processing since the aldehyde, if present in the film, would react with the color formers, e.g. as described in U.S. Pat. 3,168,406.

Once the excess aldehyde has been removed, the film may then be color-developed, fixed and stabilized, i.e. color processed, using standard procedures, such as described in U.S. Pats. 3,232,761 and 3,168,400.

The development of the negative silver image, i.e. the first development, can be accomplished using standard developer systems in which the developer is most commonly hydroquinone, but may also be other hydroquinone derivatives or equivalent compounds. Exemplary developers include phenylhydroquinone, chlorohydroquinone, dichlorohydroquinone, tetrachlorohydroquinone, bromohydroquinone and similar such organic developers. A particularly effective developer in rapid developing of the negative silver image is methylhydroquinone which, in comparison to hydroquinone, provides a much faster combination with "Metol" (methyl-para-aminophenol sulfate) and/or "Phenidone" (1-phenyl-3-pyrazolidone). A particularly effective combination is methylhydroquinone and "Phenidone" which gives fast, efficient development. For optimum results, methylhydroquinone should be employed at a pH value between 9.5 and 10.5 but preferably at a pH of 10. The preferred concentration of methylhydroquinone is from about 4 to about 13 grams/liter of developer solution. When methylhydroquinone is used with "Phenidone," the concentration of "Phenidone" is preferably from about 0.5 to about 6 grams/liter of developer solution.

The developer solution may contain accelerators (such as diamines, catechol, aliphatic amines or quaternary ammonium salts), water-softener, sodium sulfite as stabilizer, soluble thiocyanates and buffer (to control the solution to the desired alkaline pH) all of which are known in the art. The pH of the developer should be sufficiently alkaline to ionize the developer but not too alkaline to avoid film emulsion damage.

Where high energy developer systems are employed, anti-fogging agents are advantageously employed to minimize fogging of the emulsion, particularly in the outer layer. Suitable anti-fogging agents are known in the art (vide: U.S. Pat. 3,295,976).

The temperature at which the first development should be conducted must be limited to just below the minimum film reticulation temperature, i.e. the temperature at which the emulsion undergoes damage. Usually, temperatures at or near room temperature ranging to 75° F. or slightly higher may be used with commonly available three layer film.

After the first development, the film is then treated in an acid stop bath for a time sufficient to acidify the emulsion. If not acidified, the emulsion being alkaline from the first development step, the aldehyde hardner will react with the color couplers in the emulsion and thus reduce the amount of color coupler available for the color-forming development step. The adjustment of the film emulsion to acid pH prevents such reaction as is known in the art. It has been surprisingly found that the use of swell-suppressing agents in the acid stop bath improves the efficiency of the acidification, and also facilitates passage of the undesirable developer and oxidized developer into the acid stop bath.

The swell-suppressing agents include a variety of inorganic compounds, especially soluble sulfate, nitrate and phosphate salts such as alkali metal or ammonium salts. Especially effective are alkali metal sulfates or ammonium sulfate. Of these, sodium sulfate is preferred due to its ready availability. The amount of salt employed usually ranges from about 20 g. to about 100 g. per liter of stop bath solution. The amount is not critical as long as sufficient quantity to suppress the film swelling is employed. Such amount is readily determinable by routine testing. The aforementioned range will include the most commonly

effective amounts, which amounts of course are dependent on the nature of the film emulsion.

The stop bath usually contains an organic acid in an amount to provide a pH in the range of about 4 to 6 and may include buffer salts to insure maintenance of the desired pH value. Most commonly, acetic acid is employed because of its availability and economy but other such acids may be used, e.g. citric acid, propionic, gluconic, and the like.

The length of time required for exposure of the film to the acid stop bath will vary from two to four minutes, but when the swell-suppressing agent is present, the residence time required is materially shortened, thus minimizing the possible deleterious effect of the acetic acid on the color materials in the layers of the emulsion. For example, with the swell-suppressing agents in the acid stop bath, a period of about 30 seconds is all that is required to render the film emulsion acidic. In addition, it is found that a better maximum density is obtained in the color film eventually developed when the swell-suppressing agent is employed in the acid stop bath.

The aldehyde hardening step is accomplished by immersing the film in an aqueous solution of the aldehyde hardner at a concentration of at least 1%, the actual concentration being determined by the individual aldehyde selected and the degree of hardness required. The hardners are useful in acid or neutral solution, but are preferably used at acid pH values, usually not lower than a pH of 4.

Some aldehydes are not as effective as others, as might be expected. The most effective are dialdehydes and, especially glutaraldehydes, such as glutaraldehydes, beta-methyl-glutaraldehyde; alpha, alpha-dimethylglutaraldehyde, alpha-methylglutaraldehyde, and alpha, beta-dimethylglutaraldehyde. In general, the hardening procedure is known to the art and has been described in the literature, e.g. U.S. Pats. 3,232,761 and 3,168,400. Other aldehydes may be employed, e.g. succinaldehyde, formaldehyde, and combinations of these.

In the present process it is preferred to treat the film with the aldehyde solution at an initial temperature ranging up to 100° F. although higher temperatures are possible. A particularly preferred temperature is about 100° F. at which a thirty second treatment provides excellent results. In this step, the use of higher temperature may lead to emulsion damage if only in the initial immersion. Since at 100° F. a period of only 30 seconds provides optimum results, the use of higher temperatures is not necessary and is avoided particularly because of possible deleterious effects to the emulsion.

The film may be processed with the aldehyde hardner immediately after the acid stop bath treatment with no intervening washing step.

As has been previously mentioned, the emulsion is treated in the hardening step to make it stable to water at a temperature of at least 140° F., and preferably 180° F. This limitation is a measure of the amount of hardening required, and is not intended to specify processing temperatures for steps subsequent to hardening.

After the hardening step, as previously mentioned, the excess aldehyde in the emulsion must be removed before the color processing steps since carryover of the aldehyde will result in undesirable side reactions, and diminish color formation. The aldehyde may be removed by reaction with aldehyde reactive compounds, such as aldehyde-reactive amines by the method described in U.S. Pat. 3,168,400, which is incorporated herein by reference.

The color developing step is accomplished by art recognized methods any of which can be employed in the present process.

The subsequent processing steps of bleaching, fixing, and stabilizing can be done by art-recognized procedures.

A particularly effective fixing solution is one comprising a mixture of a soluble thiocyanate and a soluble thiosulfate which gives rapid and efficient fixing. The soluble

forms of each of the salts embrace the ammonium salt and alkali metal salts, especially the sodium salts which are most readily available and thus preferred. A particularly effective mixture of the fixing agents is a molar ratio of 1 mole of thiocyanate to 3 moles of thiosulfate, which gives best results.

As is generally known, after bleaching and fixing, the film is stabilized by treatment with known stabilizers, most commonly formaldehyde. It has been unexpectedly found that the addition of chelating agents to the stabilizing solution eliminates sludge and scum formation which is often noted in developed color film, particularly when processed at higher than room temperature after use of the aldehyde hardeners. For example, a formaldehyde stabilizer solution showed heavy sludge formation in a short time of use, e.g. after processing about 2 square feet of film. The addition of a chelating agent substantially prevented sludge formation until the reagent became spent.

The chelating agents are assumed to react with dissolved iron, in the form of Fe(II) and Fe(III), and silver ions, solubilizing these in the form of soluble chelate compounds. This assumption is not meant to be binding but is offered as a possible explanation. The chelating agents are those which, in fact, do form soluble chelate compounds with metallic ions and include ethylenediaminetetraacetic acid and ethylenetriaminepentacetic acid, inorganic salts such as soluble phosphates, e.g. tetrasodium pyrophosphate, and organic acids, such as gluconic acid and heptanoic acid. Of course, the chelating agent selected should not react in an adverse way with the film or the stabilizer under the conditions of use, i.e., they should be photographically-compatible.

The amount of chelating agent can vary substantially and will be determined by the needs of any process. In batch treatment methods, more concentrated solutions up to the limit of solubility of the chelating agent would be employed. In automated processing, any convenient concentration may be maintained by automatic replenishment systems. The required concentrations of chelating agent may be determined by routine experimentation. In replenishment systems, the usual concentration of chelating agent is approximately from 5 to 20 grams per liter, with about 10 grams per liter being preferred.

The problem of sludge formation which clogs tanks and lines in automatic processing apparatus and necessitates frequent change of stabilizer solution is essentially obviated by the aforementioned use of chelating agents. In normal use, the stabilizer remains sludge free and useful until the effective chelating capacity is exhausted.

As previously mentioned, hardening of the emulsion subsequent to silver negative development is preferably accomplished with dialdehyde hardners, especially a glutaraldehyde hardener which permits the use of higher temperatures than previously possible in the various steps of color-processing, i.e. color-developing, stopping the color developer, bleaching, fixing and stabilizing. Temperatures well in excess of 100° F. can be employed, ranging up to about 180° F. and even higher. For practical purposes, temperatures in the range of from about 140° to about 155° F. are preferred since these temperatures give optimum results and are especially suited for automatic film processing equipment.

As will be appreciated by those in the art, the use of high temperatures permits more rapid processing since it reduces the time requirements for the various steps of reversal color processing, thus reducing the overall time required for processing an exposed color film to a color image. For example, when the color-processing steps are conducted at a temperature of 145° F. the total processing time is reduced to as little as 5 minutes, or slightly less than 5 minutes.

#### NEGATIVE COLOR PROCESSING

In contrast to reversal color processing, negative color processing involves a first development with a color-

forming developer in which the negative silver image and color image are simultaneously formed. The color-forming developers used and the methods of developing are well-known in the art and are those mentioned in connection with the color development step of reversal color processing.

For rapid negative processing, the developing step is conducted at temperatures below the minimum film reticulation temperature. Usually, temperatures at or near room temperature ranging to 75° F. or slightly higher may be used with commonly available three layer film. The developing is stopped as desired by treatment of the developed film with art-recognized clearing baths, after which the film is then hardened as described herein for color reversal processing.

The hardening treatment and the subsequent processing steps of bleaching, fixing and stabilizing are accomplished using the same procedures as hereinbefore described in connection with the color reversal processing. However, combination of steps is possible. For example, bleaching and fixing can be effected by using a combined bleach-fixing bath which combined bath usually requires from about 45 seconds to about 60 seconds. If the hardening step is conducted at alkaline pH, the stabilizing step may be omitted, in which case, the chelating agent normally used in the stabilizer solution can be included in the fixing solution, even when combined with the bleaching solution.

In general, the procedures, including the temperature and time for the various steps of negative color processing are the same as for reversal color processing. One exception is the time required for negative development where usually from about two to about 2.5 minutes is necessary.

As in reversal color processing, hardening of the color film prior to negative development gives the same difficulty with color balance since the sensitometric quality of the film is permanently set in the first development step.

In some instances, both the rapid reversal color process and the rapid negative color process described herein can be improved by using one or more viscous processing solutions. Any number of the liquid process solutions used for either of these color processes can be made viscous by the addition of small amounts of one or more thickeners.

It has been found that the shelf life of color processing solutions, normally very short with liquids because of their complex nature, can be doubled or improved even more by making them viscous.

Additionally, it is much more economical to use viscous color processing solutions than their nonviscous counterparts. This is partly because the complex formulations can be simplified, as for example by omitting buffers and using smaller amounts of sulfites which are required in liquids to prevent aerial oxidation of various processing agents. It is also possible when using viscous solutions in some cases to eliminate certain processing solution entirely. Washes heretofore used between processing solutions can be eliminated. Another factor contributing to make viscous processing solutions more economical than their liquid counterparts is the fact that more efficient use of the active ingredients can be accomplished by using just the proper amount of agent in each viscous layer applied to the film. This is not possible, of course, when liquid baths are used to continuously process large volumes of film because such baths require replenishment systems which result in the waste of good chemistries through the overflow.

Other advantages resulting from the use of viscous processing solutions in contrast to normal liquid solutions include the lower cost of maintaining elevated temperatures of the thin viscous layers for rapid processing and the use of less complex and more economical processing equipment made possible by the elimination of the need processing tanks, agitation devices and replenishment systems.

Furthermore, it is possible to process at higher tem-

peratures using viscous processing solution without encountering the problems normally encountered with liquids at elevated temperatures such as film reticulation and softening of the photosensitive emulsion. Processing temperatures of up to about 150° F. or more can be used. Higher processing temperatures, of course, result in faster processing rates which are always welcome in color film processing.

Additionally, it is not necessary to maintain large volumes of solutions at high temperatures when viscous solutions are used. This reduces the power required for operating automatic processing equipment and also eliminates many of the other problems associated with having to maintain large volumes of photographic processing chemistries at very high temperatures.

Standard color processing liquids are made viscous by adding one or more special thickeners. The term thickeners is used to describe a class of chemical agents which cause the processing liquids to become very viscous when small amounts are added. In general, these agents should provide the processing liquids with a viscosity in the range of from about 100 to about 50,000 centipoises measured at 80° F. with a viscometer such as a Brookfield viscometer when an amount of agent of 5% by weight or less based on the total weight is added to the processing liquids. Preferably, amounts of up to about 5% of the agent will provide the processing solutions with viscosities in the range of from about 1,000 to about 20,000 centipoises measured at 80° F.

Some examples of preferred thickeners because of the good results they produce include the following:

| Trade name    | Generic name                 | Source                                   |
|---------------|------------------------------|------------------------------------------|
| Gendriv 492   | Natural gum                  | General Mills, Inc., Minneapolis, Minn.  |
| Jaguar A-20-A | Guar bean gum                | Stein, Hall & Co., Inc., New York, N.Y.  |
| Kelzan F      | Xanthan gum                  | Kelco Co., San Diego, Calif.             |
| Manucol SA/LM | Sodium alginate derivative   | Marine Colloids, Inc., Springfield, N.J. |
| Algin P932    | do                           | Do.                                      |
| Manutex RS    | do                           | Do.                                      |
| SA-1291.1     | Sodium polystyrene sulfonate | Dow Chemical Co., Midland, Mich.         |
| Polymer 705D  | Guar bean gum                | Stein, Hall & Co., Inc., New York, N.Y.  |

As can be seen, naturally occurring substances such as polysaccharides and synthetic polymers such as polystyrenes can be used as thickeners providing they meet the criteria set out above. Many other thickeners will be known or ascertainable by routine experimentation to those skilled in the art.

The above discussion is not meant to indicate that all of the thickeners mentioned or all of those known by others can be used in each and every color processing solution, or should be used in each and every processing solution. There are several criteria that should be followed in selecting a particular thickener or combination of thickeners for the specific color processing liquid under consideration. These criteria include: inertness over the operative pH range in the presence of the anions and cations in solution; ability of the viscous solution to resist chemical breakdown of the viscous agent due to oxidation or bacterial action; and, good mixing characteristics. These and other criteria which are well known to those skilled in the art will require only routine experimentation to apply before a particular thickener or combination of thickeners is selected for a specific color processing liquid.

Apparatus for continuously and automatically carrying out the rapid color processes described herein is illustrated in FIGS. 1-3.

FIG. 1 illustrates a deep tank continuous processor suitable for practicing the rapid reversal color process described herein. An unprocessed reversal film 2, previously exposed, enters the processor by entrance transport roller

4 and is thereafter conveyed by a sequence of transport rollers 5 and turnaround rollers 9 through a series of processing solutions contained within the various tanks of the processor. Processed reversal color film 3 exits from the processor by means of exit transport roller 7. The transport rollers 4, 5 and 7 are driven by suitable means such as a chain drive.

As can be seen, the processor has tanks respectively containing: first developer 6, stop bath 8, hardener 10, neutralizer 12, color developer 14, clearing bath 16, bleach 18, fixing bath 20, wash 22, and stabilizer 24. A dryer 26 is provided after stabilizer 24. Suitable solutions for each of the tanks are described in Example 1. The time of processing for each of the solutions is determined by the path length of the film in each tank. The path length can be suitably adjusted by varying the number and length of up and down traverses the film makes in each tank.

While the solutions require special materials of construction, these are well known in the photographic processing art.

Where there is a large temperature differential between adjacent tanks, it is desirable to provide thermally insulated walls between such tanks. In the apparatus shown in FIG. 1, for example, insulated walls 28, 30 and 32 are used to respectively separate stop bath 8 from hardener 10; neutralizer 12 from color developer 14; and stabilizer 24 from the drying section 26.

Since hardening is often accomplished with aldehydes which tend to give off noxious vapors, hardener tank 10 is provided with a cover 34 to prevent leakage of these vapors and a vent 36.

FIG. 2 illustrates an apparatus suitable for processing a negative color film using the rapid process described herein. An exposed, unprocessed negative color film 50 is introduced into the apparatus by entrance transport roller 52 and is subsequently conveyed through a series of processing tanks by transport rollers 53 and turn-around rollers 57. The length of time that the film is exposed to each processing solution is determined by the number and length of up and down traverses the film makes on rollers 53, 57 in each tank. Fully processed negative color film 51 exits from the processor by means of exit transport roller 55.

The processor is divided into a number of tanks containing respectively: color developer 54, clearing bath 56, hardener 58, bleach 60, fixing bath 62, wash 64, and stabilizer 66. A dryer 68 is provided after stabilizer 66. Suitable processing solutions can be found in Example 7. The respective tanks require special materials of construction because of the corrosive chemicals contained in many of these solutions, but these are well known to those skilled in the photographic processing art.

Where a significant temperature differential exists between adjacent processing solutions, the apparatus is provided with thermally insulated walls therebetween such as walls 70 and 72 separating the clearing bath 56 from the hardening bath 58 and the stabilizer 66 from the drying section 68.

FIG. 3 illustrates another embodiment of a processing apparatus for rapidly procesing reversal color film by a modified process as described herein. Unprocessed, exposed reversal color film 100 is introduced to the processor by entrance transport roller 101. The fully processed film 102 exits from the machine by means of exit transport roller 103. In the apparatus, the partially processed film is transported through a series of tanks containing the required processing solutions by transport rollers 104 and turn-around rollers 105.

The processor is divided into a series of tanks respectively containing: first developer 106, stop bath 108, hardener 110, neutralizer 112, color developer 114, water wash 116, clearing bath 118, bleach 120, fixing bath 122, wash 124, and stabilizer 126. A dryer 128 is provided after stabilizer 126.

In this apparatus, a viscous color developer solution is used to color develop the film rather than the normal color developer. Viscous color developer is extruded onto the exposed film surface by extrusion head 130. Color development section 114 of the processing apparatus does not contain processing solution, of course, but merely contains moist air at an elevated temperature, preferably about 150° F. After a layer of viscous color developer has been extruded onto the film surface, the film passes down towards the bottom of color development section 114 and around reversing transport roller 132 which flips the film over so that the viscous layer remains on the top surface as the film travels back towards the top of color development section 114. After color processing is complete, viscous color developer is removed from the film in water wash section 116 by a series of water sprays 134 before the film enters the next tank containing clearing bath 118.

Processing apparatus using viscous color development has the advantage that a large tank of color developer does not have to be maintained at a high temperature thereby lessening power requirements and simplifying processing.

As should be obvoius to those skilled in the art, the aforementioned improved acid stop bath for the first developer, i.e. silver negative developer, is useful not only in rapid processing of color reversal film but also in normal color processing in general, as is true of the stabilizer solution containing chelating agent, and the sulfate-containing stopbath. The developer solution containing methylhydroquinone is also useful in normal color processing as well as in processing of black and white film.

Multi-layer films of the type which can be employed in the present invention are well known in the art and have been described in the patent literature, such as U.S. Pats. 2,322,027; 2,252,718; the aforementioned 3,168,400 and 3,232,761; and 3335,004, among others.

The following examples further illustrate the invention.

#### EXAMPLE 1

40 A three-color silver bromoiodide film wherein gelatin is employed as the hydrophilic colloid and wherein cyan, magenta and yellow color formers of the type described in U.S. Pat. 2,322,027, mentioned above, are incorporated in the emulsions, is exposed for 1/50 second to a 500-watt tungsten lamp, adjusted to a color temperature of 6100° K. in an intensity scale sensitometer, and then treated in 45 a developer having the following composition:

|                                                      |       |      |       |
|------------------------------------------------------|-------|------|-------|
| Quadrafos (sodium tetraphosphate-sequestering agent) | ----- | g--  | 2.0   |
| Phenidone                                            | ----- | g--  | 6.0   |
| Sodium sulfite (anhydrous)                           | ----- | g--  | 25    |
| Methylhydroquinone                                   | ----- | g--  | 7.0   |
| Ethylenediamine (93%)                                | ----- | ml-- | 26.0  |
| Sodium thiocyanate                                   | ----- | g--  | 1.0   |
| Potassium iodide (0.1% solution)                     | ----- | ml-- | 13    |
| 55 Antifogging agent (0.05%) solution                | ----- | ml-- | 5.36  |
| Boric acid (to pH 10.0)                              | ----- | g--  | 10-20 |
| H <sub>2</sub> O to make one liter.                  |       |      |       |

The solution is maintained at 75° F. and the total treatment time is 70 seconds.

60 The developed film is immersed in a stopbath maintained at 75° F. for a period of 30 seconds and having the following composition:

|                                     |       |      |       |
|-------------------------------------|-------|------|-------|
| Acetic acid (glacial)               | ----- | ml-- | 20    |
| Sodium acetate                      | ----- | g--  | 10.5  |
| Sodium sulfate                      | ----- | g--  | 100.0 |
| H <sub>2</sub> O to make one liter. |       |      |       |

70 Without intervening washing, the film is next treated in a hardening bath maintained at 100° F. for a period of 10 seconds and having the following compositions:

|                                     |       |      |     |
|-------------------------------------|-------|------|-----|
| Glutaraldehyde (25% solution)       | ----- | ml-- | 80  |
| Sodium sulfate (anhydrous)          | ----- | g--  | 100 |
| H <sub>2</sub> O to make one liter. |       |      |     |

75 pH adjusted to 4.0.

11

The hardened film is then immersed in an aldehyde neutralizer both maintained at 100° F. for 10 seconds and having the following composition:

Hydroxyamine sulfate ----- g. 20.0 5  
 Sodium sulfate (anhydrous) ----- g. 50.0  
 Acetic acid (glacial) ----- ml. 10.0  
 H<sub>2</sub>O to make one liter.

The film is next immersed for 36 seconds at 145° F. 10 in a color developer having the following composition:

Quadrafos ----- g. 5.0  
 Benzyl alcohol ----- ml. 15.0  
 Tertiary butylamine borane ----- g. 0.28 15  
 Sodium sulfite (anhydrous) ----- g. 7.5  
 Trisodium phosphate ----- g. 40.0  
 Sodium bromide ----- g. 0.9  
 Potassium iodide (0.1% solution) ----- ml. 31.0  
 Citrazinic acid ----- g. 3.6 20  
 4-amino - N - ethyl-N-(beta-methanesulfonamidoethyl)-m-toluidine sesquisulfate monohydrate ----- g. 13.0  
 Sodium hydroxide ----- g. 7.5  
 H<sub>2</sub>O to make one liter.

After development, the film is immersed for 10 seconds 25 at 145° F. in a clearing bath composed of sodium metabisulfite (40.0 g. per liter of water) and then bleached for 40 seconds at 145° F. in a solution composed of:

Potassium ferricyanide ----- g. 120 30  
 Sodium bromide ----- g. 40  
 Borax ----- g. 1  
 Carbowax (polyethyleneglycol) (50% solution) ----- ml. 10  
 Sodium hydroxide ----- g. 3 35  
 H<sub>2</sub>O to make one liter.  
 pH adjusted to 7.85±0.1.

The film is then fixed by immersion for 25 seconds at 40 145° F. in a fixing bath composed of:

G.  
 Ammonium thiocyanate ----- 250  
 Sodium thiosulfate (anh.) ----- 150  
 Sodium sulfite ----- 20  
 Boric acid ----- 7.5 45  
 Sodium metabisulfite ----- 20  
 H<sub>2</sub>O to make one liter.

Finally, the film is stabilized by treatment for 15 seconds at 145° F. in a solution composed of:

Formalin ----- ml. 10 50  
 Ethylene diaminetetraacetic (tetra sodium salt) ----- g. 10  
 H<sub>2</sub>O to make one liter.

The total processing time is 266 seconds. Good sensitometric results are obtained.

#### EXAMPLE 2

A strip of Ektachrome type 2448 film is exposed on an Eastman Kodak Ib sensitometer with a Corning 5900 daylight filter, to 21 step carbon wedge for 1/25 second. After exposure the strip is processed according to the following sequence:

Developer: 75° F. for 70 seconds  
 Stop bath: 75° F. for 30 seconds  
 Hardener: 100° F. for 30 seconds  
 Neutralizer: 100° F. for 10 seconds  
 Color developer: 145° F. for 35 seconds  
 Clear: 145° F. for 10 seconds  
 Bleach: 145° F. for 40 seconds  
 Fixer: 145° F. for 25 seconds  
 Rinse: 145° F. for 10 seconds  
 Stabilizer: 145° F. for 15 seconds.

12

Developer:  
 Quadrafos ----- g. 2.0  
 Phenidone ----- g. 1.0  
 Sodium sulfite (anh.) ----- g. 25.0  
 Methylhydroquinone ----- g. 7.0  
 Ethylenediamine (93%) ----- ml. 26.0  
 Sodium thiocyanate ----- g. 1.0  
 Boric acid ----- g. 12.0  
 Potassium iodide (0.1% soln.) ----- ml. 13.0  
 1 - phenyl-2-tetrazoline-5-thione (0.5% soln.) ----- ml. 5.0

Water to make 1.0 liter.

Stop bath:

Sodium sulfate ----- g. 100.0  
 Acetic acid (glacial) ----- ml. 20.0  
 Sodium acetate (3H<sub>2</sub>O) ----- g. 10.5  
 Water to make 1.0 liter.

Hardener:

Glutaraldehyde (25% soln.) ----- ml. 80  
 Sodium sulfate (anh.) ----- g. 100  
 H<sub>2</sub>O to 1.0 liter.  
 pH 4.0.

Neutralizer:

Hydroxylamine sulfate ----- g. 20.0  
 Sodium sulfite (anh.) ----- g. 50.0  
 Acetic acid (glacial) ----- ml. 10.0  
 H<sub>2</sub>O to 1.0 liter.

Color developer:

Quadrafos ----- gms. 5.0  
 Benzyl alcohol ----- ml. 15.0  
 tert-Butylamine borane ----- gms. 0.28  
 Sodium sulfite (anh.) ----- gms. 7.5  
 Sodium phosphate (tribasic) ----- gms. 40.0  
 Sodium bromide ----- gms. 0.9  
 Potassium iodide (0.1%) ----- ml. 31.0  
 Citrazinic acid ----- gms. 3.6  
 4 - amino-N-ethyl-N-(beta-methanesulfonamidoethyl) - m - toluidine, sesquisulfate monohydrate ----- gms. 13.0  
 Sodium hydroxide ----- gms. 7.5  
 H<sub>2</sub>O to 1.0 liter.  
 pH 12.0.

Clearing bath:

Potassium metabisulfite ----- gms. 40.0  
 H<sub>2</sub>O to 1.0 liter.

Bleach:

Sodium bromide ----- gms. 26.0  
 Sodium ferrocyanide (10H<sub>2</sub>O) ----- gms. 180.0  
 Potassium persulfate ----- gms. 51.0  
 Sodium phosphate (dibasic anh.) ----- gms. 12.5  
 Carbowax 1540 (50%) ----- ml. 6.0  
 H<sub>2</sub>O to 1.0 liter.  
 pH 7.8.

Fixer:

Sodium sulfite ----- g. 10  
 Sodium thiosulfate (5H<sub>2</sub>O) ----- g. 250  
 Ammonium sulfate ----- g. 50

Stabilizer:

Formalin solution ----- ml. 10  
 Ethylenediamine tetraacetic acid (tetra sodium salt) ----- g. 10.0  
 Water to make 1.0 liter.

Good sensitometric results are obtained, as evidenced by the good color balance as shown in the sensitometric curves of FIG. 4.

#### EXAMPLE 3

A strip of Ektachrome 2448 exposed as described in Example 2 is processed similarly except that in place of methylhydroquinone an equal molar concentration of hydroquinone was used (6.2 grams/l). The sensitometric results indicate that photographic speed decreased 50%

## 13

(1 f stop) for all three dyes; a 25% increase of development time is required to restore the speed.

## EXAMPLE 4

A strip of Ektachrome type SO-271 is exposed as in Example 2 for  $\frac{1}{10}$  second and processed as in Example 2 except the stop bath did not contain sodium sulfate. The maximum density obtained with magenta dye decreased 0.3 density units.

## EXAMPLE 5

A strip of exposed Ektachrome type SO-271 is hardened and neutralized prior to the first developer (pre-hardened) which is followed by the stop bath, color developer, and the remainder of the process in Example 2. Because of the silver halide fogging property of aldehyde hardeners the sensitometric results indicates serious dye density losses. The addition of two antifogging agents: 3 mg./l. 1-phenyl-2-tetrazoline-5-thione and 20 ml./l. N-methyl benzothiazolium p-toluene sulfonate to the hardener and the addition of 17 gm./l. sodium bromide to the neutralizer restored the dye densities. However, color balance is seriously modified, as evidenced by lack of good color balance. Attempts to restore proper color balance by varying the first developer time are unsuccessful.

## EXAMPLE 6

The procedure of Example 2 is repeated except the stabilizer does not contain E.D.T.A. 4 Na. After several strips have been processed, a precipitate and a colloidal suspension formed in the stabilizer. All strips upon drying form a scum on the surfaces of the film. This does not occur when EDTA 4 Na is present in the stabilizer.

## EXAMPLE 7

A strip of Ektacolor Print film is exposed on an Eastman Kodak 1B sensitometer to a 21 step carbon wedge for 1 second with filtration to obtain a neutral image (.20 magenta+.50 yellow+Wratten 2B+Kodacolor Negative mask). After exposure the film is processed according to the following schedule:

Developer: 75° F. for 3 minutes

Clear: 75° F. for 30 seconds

Hardener: 100° F. for 30 seconds

Bleach: 150° F. for 30 seconds

Fixer: 150° F. for 25 seconds

Rinse: 150° F. for 10 seconds

Stabilizer: 150° F. for 15 seconds

Developer:

|                                                                                             |    |      |
|---------------------------------------------------------------------------------------------|----|------|
| Benzyl alcohol                                                                              | ml | 9.0  |
| Benzotriazole                                                                               | g  | 0.05 |
| 6-nitrobenzimidazole nitrate                                                                | g  | 0.05 |
| Sodium sulfate (anh.)                                                                       | g  | 2.5  |
| 4 - amino-N-ethyl-N-(betamethanesulfonamidoethyl) - m - toluidine sesquisulfate monohydrate | g  | 12.0 |
| Sodium metaborate                                                                           | g  | 40.0 |
| Sodium phosphate tribasic                                                                   | g  | 20.0 |
| Potassium bromide                                                                           | g  | 1.2  |
| Sodium hydroxide                                                                            | g  | 4.0  |
| pH 11.7.                                                                                    |    |      |

Clear:

|                                |   |      |
|--------------------------------|---|------|
| Potassium metabisulfite        | g | 80.0 |
| H <sub>2</sub> O to 1.0 liter. |   |      |

The remaining solutions are identical to those for reversal processing described in Example 2. Good sensitometric results are obtained as shown in FIG. 5.

## EXAMPLE 8

The procedure of Example 7 is repeated except that the developing is carried out at 100° F. for 1 minute and clearing at 100° F. for 30 seconds. Good sensitometric

## 14

results are obtained. However, emulsion reticulation occurs.

## EXAMPLE 9

The procedure of Example 7 is repeated except the hardening step precedes the development step, according to the following schedule:

|    |                                     |
|----|-------------------------------------|
| 10 | Hardener: 100° F. for 30 seconds    |
| 10 | Neutralizer: 100° F. for 10 seconds |
| 10 | Developer: 150° F. for 30 seconds   |
| 10 | Clear: 150° F. for 10 seconds       |
| 10 | Bleach: 150° F. for 30 seconds      |
| 15 | Fixer: 150° F. for 25 seconds       |
| 15 | Rinse: 150° F. for 10 seconds       |
| 15 | Stabilizer: 150° F. for 15 seconds  |

The results indicate serious fogging of the magenta and yellow layer, while underdevelopment of the yellow layer also occurs. The addition of organic antifoggants to the hardener (3 mg./l. 1-phenyl-2-tetrazoline-5-thione and 20 mg./l. N-methyl benzothiazolium p-toluene sulfonate) reduces the fog level considerably. However, the sensitometric results shown in FIG. 6 indicate a still excessive fog level for magenta and very serious underdevelopment of the yellow layer. Further attempts to restore good color balance when the hardener is used prior to development are equally unsuccessful.

## EXAMPLE 10

The procedure of Example 2 is repeated with diethylenetriamine pentacetic acid, in lieu of ethylenediamine tetraacetic acid with similar results. Similarly tetrasodium pyrophosphate, gluconic acid and heptanoic acid are substituted for ethylenediamine tetracetic acid with similar results.

## EXAMPLE 11

The following rapid reversal color process solutions are prepared by first preparing the processing liquid and then mixing in the specified thickeners until the solution is viscous and homogeneous:

|    |                                      |
|----|--------------------------------------|
| 45 | First developer:                     |
| 45 | Sodium sulfate ----- g 75            |
| 45 | EDTA ----- g 2                       |
| 45 | Phenidone ----- g 1                  |
| 45 | Hydroquinone ----- g 30              |
| 45 | Sodium hydroxide ----- g 25          |
| 50 | Thymol <sup>1</sup> ----- ml 5       |
| 50 | H <sub>2</sub> O to 1 liter.         |
| 50 | Kelzan F (thickener) ----- g 5       |
| 50 | Manucol SA/LM (thickener) ----- g 25 |
| 55 | Viscosity 12,600 centipoises.        |
| 55 | pH 12.5.                             |

First stop bath:

|    |                                           |
|----|-------------------------------------------|
| 60 | Thymol <sup>1</sup> ----- ml 5            |
| 60 | Sodium sulfate (anhedrous) ----- g 100    |
| 60 | Acetic acid (glacial) ----- ml 20         |
| 60 | Sodium acetate (crystalline) ----- g 10.5 |
| 60 | H <sub>2</sub> O to 1 liter.              |
| 60 | Kelzan F ----- g 5                        |
| 60 | Manucol SA/LM ----- g 25                  |
| 65 | Viscosity, 8,300 centipoises.             |
| 65 | pH 4.0.                                   |

Hardener:

|    |                                          |
|----|------------------------------------------|
| 70 | Thymol <sup>1</sup> ----- ml 5           |
| 70 | Glutaraldehyde (25 percent) ----- ml 160 |
| 70 | Sodium sulfate (anhedrous) ----- g 100   |
| 70 | H <sub>2</sub> O to 1 liter.             |
| 70 | Kelzan F ----- g 4                       |
| 70 | Manucol SA/LM ----- g 24                 |
| 75 | Viscosity 10,800 centipoises.            |
| 75 | pH 4.0.                                  |

## Neutralizer:

|                               |     |    |
|-------------------------------|-----|----|
| Thymol <sup>1</sup>           | ml. | 5  |
| Hydroxylamine sulfate         | g.  | 20 |
| Acetic acid (glacial)         | ml. | 10 |
| NaOH                          | g.  | 10 |
| H <sub>2</sub> O to 1 liter.  |     | 5  |
| Kelzan F                      | g.  | 5  |
| Manucol SA/LM                 | g.  | 30 |
| Viscosity 10,300 centipoises. |     |    |
| pH 6.0.                       |     | 10 |

## Color developer:

|                              |        |     |
|------------------------------|--------|-----|
| Thymol <sup>1</sup>          | ml.    | 5   |
| Quadrafos                    | g.     | 5   |
| Benzyl alcohol               | ml.    | 15  |
| T-butylamine borane          | tablet | 1/2 |
| Sodium sulfite               | g.     | 7.5 |
| Sodium phosphate (tribasic)  | g.     | 40  |
| Sodium bromide               | g.     | 0.9 |
| KI (0.1% solution)           | ml.    | 24  |
| Citrazinic acid              | g.     | 3.6 |
| CD-3                         | g.     | 13  |
| NaOH                         | g.     | 7.5 |
| H <sub>2</sub> O to 1 liter. |        |     |
| Kelzan F                     | g.     | 1.5 |
| Manucol SA/LM                | g.     | 60  |
| Viscosity 8,300 centipoises. |        | 25  |
| pH 12.3.                     |        |     |

## Second stop bath:

|                              |     |    |
|------------------------------|-----|----|
| Thymol <sup>1</sup>          | ml. | 5  |
| Sodium metabisulfite         | g.  | 40 |
| H <sub>2</sub> O to 1 liter. |     | 30 |
| Kelzan F                     | g.  | 5  |
| Manucol SA/LM                | g.  | 10 |
| Viscosity 3,300 centipoises. |     |    |
| pH 4.0.                      |     | 35 |

## Bleach:

|                                       |     |      |
|---------------------------------------|-----|------|
| Thymol <sup>1</sup>                   | ml. | 5    |
| Sodium bromide                        | g.  | 26   |
| Sodium ferrocyanide, dehydrate        | g.  | 180  |
| Potassium persulfate                  | g.  | 51   |
| Sodium phosphate, dibasic (anhydrous) | g.  | 12.5 |
| Carbowax 1540 (50 percent)            | ml. | 40   |
| H <sub>2</sub> O to 1 liter.          |     | 6    |
| Kelzan F                              | g.  | 3    |
| Manucol SA/LM                         | g.  | 25   |
| Viscosity 8,600 centipoises.          |     | 45   |
| pH 7.8.                               |     |      |

## Fixer:

|                                  |     |     |
|----------------------------------|-----|-----|
| Thymol <sup>1</sup>              | ml. | 5   |
| Sodium thiosulfate, pentahydrate | g.  | 250 |
| Ammonium sulfate                 | g.  | 50  |
| Sodium sulfite                   | g.  | 10  |
| H <sub>2</sub> O to 1 liter.     |     |     |
| Kelzan F                         | g.  | 3   |
| Manucol SA/LM                    | g.  | 25  |
| Viscosity 6,600 centipoises.     |     | 55  |
| pH 7.6.                          |     |     |

## Wash stabilizer:

|                                     |       |    |
|-------------------------------------|-------|----|
| Thymol <sup>1</sup>                 | ml.   | 5  |
| Formalin                            | ml.   | 10 |
| EDTA (tetrasodium salt)             | grams | 10 |
| H <sub>2</sub> O to 1 liter.        |       | 60 |
| Kelzan F                            | grams | 4  |
| Manucol SA/LM                       | do    | 30 |
| Viscosity SA&LM 10,800 centipoises. |       | 65 |
| pH 10.0                             |       |    |

<sup>1</sup> 0.1% solution.

All pH and viscosity values are measured at 80° F. and the viscosities are measured with a Brookfield viscometer.

The viscous processing solutions are applied to the film with a thickness of about 0.02 inch by extruding them through a nozzle positioned tangential to the film and are removed after the specified dwell time by a squeegee. The film speed is set at five feet per minute.

The following Eastman Kodak Ektachrome aerial type film strips are exposed through a 21-step wedge as follows:

| Type   | Exposure conditions                                                              |
|--------|----------------------------------------------------------------------------------|
| 8442   | 0.01 secs., Eastman Type 1b Sensitometer, 5,900° K. filter.                      |
| 8443   | 0.1 secs., Eastman Type 1b Sensitometer, 5,900° K., 2,200 K., 90B, G-15 filters. |
| SO-271 | 0.1 secs., Eastman Type 1b Sensitometer, no filter.                              |
| 2448   | 0.04 secs., Eastman Type 1b Sensitometer, 5,900° K. filter.                      |

Processing conditions are:

| Viscous solution | Dwell time    | Temperature, ° F. |
|------------------|---------------|-------------------|
| First developer  | 1 minute      | 100               |
| First stop       | 30 seconds    | 100               |
| Hardener         | 30 seconds    | 120               |
| Neutralizer      | 15 seconds    | 120               |
| Color developer  | 1 1/2 minutes | 150               |
| Second stop      | 30 seconds    | 120               |
| Bleach           | 1 minute      | 150               |
| Fixer            | 30 seconds    | 150               |
| Wash stabilizer  | 30 seconds    | 150               |

Approximately 80 square feet of film can be processed per gallon of solution. The films are uniformly processed with no signs of emulsion damage. Upon completion of processing, the films are dried and sensitometrically evaluated. Good sensitometric results are obtained.

## EXAMPLE 12

A viscous negative color processing developer having the following composition is prepared:

|                                            |       |      |
|--------------------------------------------|-------|------|
| Benzyl alcohol (40 percent solution)       | ml.   | 22.0 |
| Benzotriazole (0.2 percent)                | ml.   | 25.0 |
| 6-nitrobenzamidazole nitrate (0.2 percent) | ml.   | 25.0 |
| Sodium sulfite (anhydrous)                 | grams | 2.5  |
| CD-3                                       | do    | 12.0 |
| Sodium metaborate                          | do    | 40.0 |
| Sodium phosphate, tribasic                 | do    | 20.0 |
| Potassium bromide                          | do    | 1.2  |
| Sodium hydroxide                           | do    | 4.0  |
| Carboxy methyl cellulose (thickener)       | do    | 10.0 |
| H <sub>2</sub> O to 1.0 liter.             |       |      |
| pH 11.7.                                   |       |      |
| Viscosity 10,000 centipoises.              |       |      |

The stop bath, hardener, bleach, fixer and wash stabilizer have the same compositions as in Example 11.

Eastman Kodak Kodacolor X film is exposed through a 21-step tablet on an EG&G Mark VI sensitometer for 1/100 second. The film is then processed by sequentially applying a layer of viscous solution approximately 0.02 inch thick for the dwell times and at the temperatures indicated below:

| Viscous solution | Dwell time | Temperature, ° F. |
|------------------|------------|-------------------|
| Developer        | 6 minutes  | 85                |
| Stop bath        | 30 seconds | 85                |
| Hardener         | 30 seconds | 120               |
| Bleach           | 45 seconds | 150               |
| Fixer            | 30 seconds | 150               |
| Wash stabilizer  | 30 seconds | 150               |

The film is uniformly processed without damage to the photosensitive emulsion and good sensitometric results are obtained.

What is claimed is:

1. In the color processing of an exposed photosensitive medium containing color-forming material wherein said color-forming material is processed into image form including at least the steps of hardening the emulsion and developing, the improvement which comprises:
  - (a) first developing a photographic image in said medium by treatment with a photographic developer therefore; and,
  - (b) subsequently hardening the emulsion of said medium to be stable to water at a temperature of at least about 140° F.

2. An improvement of claim 1 wherein the emulsion comprises gelatin and wherein said gelatin is hardened with an aldehyde hardener therefor.

3. An improvement of claim 2 wherein said aldehyde hardener comprises a dialdehyde hardener.

4. An improvement of claim 3 wherein the gelatin emulsion is hardened to be stable to water at a temperature of at least about 180° F.

5. An improvement of claim 4 wherein said photographic developer comprises an aqueous alkaline developer and said first developing results in a black and white photographic image.

6. An improvement of claim 5 wherein said dialdehyde hardener comprises glutaraldehyde.

7. A method for rapidly processing an exposed color reversal photosensitive emulsion, comprising:

(a) first developing a black and white negative image in said emulsion by treatment with a photographic developer therefor at a temperature below that at which emulsion damage occurs;

(b) subsequently hardening the emulsion to be stable to water at a temperature of at least about 140° F.; and thereafter,

(c) color processing said emulsion at an elevated temperature above the first development temperature.

8. A method of claim 7 wherein color development is carried out at a temperature of at least about 100° F.

9. A method of claim 7 wherein color development is carried out at a temperature in the range of from about 140° F. to about 155° F.

10. A method of claim 9 wherein said photographic developer comprises an aqueous alkaline photographic developer.

11. A method of claim 10 wherein said hardening step (b) comprises:

(a) acidifying the emulsion;

(b) contacting said acidified emulsion with an aldehyde hardener therefor; and,

(c) removing substantially all free aldehyde from said emulsion prior to color processing.

12. A method of claim 11 wherein said aqueous alkaline photographic developer contains methylhydroquinone.

13. A method of claim 12 wherein said aldehyde hardener comprises a dialdehyde containing a linear chain of 2-3 carbon atoms linking the two aldehyde groups.

14. The method of claim 13 wherein said aqueous alkaline development is conducted at a temperature in the range of from about 70° F. to about 80° F. and said developer has a pH in the range of from about 9.5 to about 10.5.

15. A method of claim 14 wherein said dialdehyde hardener comprises glutaraldehyde.

16. A method of claim 15 wherein said hardening step is conducted by contacting said emulsion with said glutaraldehyde at a temperature of from about 90° F. to about 110° F. for a period of from about 10 to about 120 seconds.

17. A method of claim 16 wherein the emulsion acidification step is conducted by contacting said emulsion with an aqueous solution of a photographically-acceptable acid, the pH of said solution being in the range of from about 4 to about 6.

18. A method of claim 17 wherein said acid comprises acetic acid.

19. A method of claim 18 wherein said emulsion comprises gelatin and said acid solution includes a gelatin swell-suppressing agent.

20. A method of claim 19 wherein said gelatin swell-suppressing agent comprises an alkali metal sulfate or ammonium sulfate.

21. A method of claim 19 said gelatin swell-suppressing agent comprises sodium sulfate.

22. A method of claim 21 wherein substantially all of the free aldehyde is removed after hardening by contacting the emulsion with a solution of an aldehyde-reactive

amine at a temperature of from about 70° F. to about 145° F. and having a pH in the range of from about 3 to about 6.

23. A method of claim 22 wherein said color processing includes the following steps:

- (a) color-developing the emulsion;
- (b) clearing the emulsion of color developer;
- (c) bleaching out the metallic silver deposits;
- (d) fixing the silver halide of the emulsion; and,
- (e) stabilizing the emulsion.

24. A method of claim 7 wherein the emulsion is hardened to be stable to water at a temperature of at least about 180° F.

25. A method of claim 24 wherein color development is carried out at a temperature in the range of from about 140° F. to about 155° F.

26. In the processing of an exposed, negative, color, photosensitive emulsion including the steps of hardening said emulsion and color-developing, the improvement comprising:

- (a) first color developing the latent image in said emulsion by treatment with a color developer; and,
- (b) subsequently hardening said emulsion to be stable to water at a temperature of at least about 140° F.

27. An improvement of claim 26 wherein said emulsion is hardened by contacting it with a solution of a dialdehyde hardener.

28. An improvement of claim 27 wherein said dialdehyde hardener comprises glutaraldehyde.

29. An improvement of claim 28 wherein said emulsion is hardened to be stable to water at a temperature of at least about 180° F.

30. In the reversal color processing of an exposed photosensitive medium including at least the process steps of hardening the emulsion, developing a black and white image, and subsequently developing a color reversal image, the improvement which comprises hardening the emulsion to be stable to water at a temperature of at least about 140° F. after developing the black and white image but prior to developing the color reversal image.

31. An improvement of claim 30 wherein said emulsion is hardened to be stable to water at a temperature of at least about 180° F.

32. An improvement of claim 31 wherein color development is carried out at a temperature of at least about 100° F.

33. An improvement of claim 31 wherein color development is carried out at a temperature in the range of from about 140° F. to about 155° F.

34. An improvement of claim 33 wherein said emulsion is hardened by contacting it with a solution of a dialdehyde hardener.

35. An improvement of claim 34 wherein said dialdehyde hardener comprises glutaraldehyde.

36. An improvement of claim 1 including the use of at least one viscous processing solution.

37. An improvement of claim 36 wherein said viscous processing solution comprises a color developer solution.

38. An improvement of claim 37 wherein said viscous processing solution contains a thickener selected from the group consisting of natural gum, guar bean gum, xanthan gum, sodium alginate, sodium polystyrene sulfonate, and combinations of these.

39. An improvement of claim 36 wherein all the solutions are viscous processing solutions.

40. An improvement of claim 26 including the use of at least one viscous processing solution.

41. In the color processing of an exposed photo-sensitive medium containing color-forming material wherein said color-forming material is processed into image form including at least the steps of hardening the emulsion and developing, the improvement which comprises:

- (a) first developing a photographic image in said medium by treatment with a photographic developer therefor; and,

19

(b) subsequently hardening the emulsion of said medium to be stable to rapid processing wherein at least one of the steps after hardening is carried out at a temperature of at least about 100° F.

20

|           |        |           |       |        |
|-----------|--------|-----------|-------|--------|
| 2,359,217 | 9/1944 | Hollander | ----- | 96—111 |
| 3,232,761 | 2/1966 | Allen     | ----- | 96—111 |
| 3,140,177 | 7/1964 | Welch     | ----- | 96—111 |

## References Cited

5 NORMAN G. TORCHIN, Primary Examiner

## UNITED STATES PATENTS

J. L. GOODROW, Assistant Examiner

|           |        |               |       |        |
|-----------|--------|---------------|-------|--------|
| 3,582,347 | 6/1971 | Holly et al.  | ----- | 96—111 |
| 2,196,226 | 1/1938 | Murray et al. | ----- | 96—55  |

U.S. Cl. X.R.

96—111